# EUROPEAN PATENT SPECIFICATION

(11) **EP 2 059 617 B1**
(45) Date of publication and mention of the grant of the patent: **05.05.2010**
(21) Application number: 07826021.3
(22) Date of filing: 13.08.2007
(51) Int. Cl.: C22B 1/24, C22C 26/00

(54) **DUAL STAGE PROCESS FOR THE RAPID FORMATION OF PELLETS**
ZWEIPHASENVERFAHREN FÜR DIE RASCHE HERSTELLUNG VON PRESSLINGEN
PROCÉDÉ EN DEUX ÉTAPES POUR LA FORMATION RAPIDE DE PASTILLES

(30) Priority: 11.08.2006 ZA 200606674
(43) Date of publication of application: 20.05.2009
(73) Proprietor: Element Six Ltd, Shannon, Clare (IE)
(72) Inventor: EGAN, David, Clare (IE); WRIGHT, Derek Norman, Cratloe, Co. Clare (IE); FLYNN, Gerald F, Co Clare (IE)
(74) Representative: Benson, John Everett
(86) International application number: PCT/IB2007/053204
(87) International publication number: WO 2008/018048

(56) References cited:
- US-A- 3 316 073
- US-B1- 6 238 280
- BURCKHARDT STEFAN: "New technique for granulating diamond and metal powders" MET POWDER REP; METAL POWDER REPORT APR 1998 ELSEVIER SCI LTD, EXETER, ENGL, vol. 53, no. 4, April 1998 (1998-04), pages 28-29, XP002464798
- TURTON R ET AL: "The scale-up of spray coating processes for granular solids and tablets" POWDER TECHNOLOGY, ELSEVIER SEQUOIA, LAUSANNE, CH, vol. 150, no. 2, 16 February 2005 (2005-02-16), pages 78-85, XP004766952 ISSN: 0032-5910

## Description

### BACKGROUND OF THE INVENTION

This invention relates to a process for the formation of pellets. In particular this application relates to a dual stage process for the formation of pellets by coating a central core with a powder material.

The process has a broad range of applications ranging from pelletising diamond seeds for High Pressure High Temperature diamond synthesis to using pelletised ultra hard materials in cutting or abrading tools.

Many high technology cutting and abrading tools are conventionally manufactured from a suitable metal with grains of ultra hard material such as diamond or cubic boron nitride embedded in the metal forming the cutting or abrading components of the tools. One option in manufacturing such tools is to initially pelletise the ultra hard material in a layer of the metal and subsequently press or sinter a plurality of these pellets into the tool components.

The oil, gas and mining industries are projected to significantly increase their demand for pelletised ultra hard products in the future. In order to maximise profitability and respond to this demand it will be necessary to have an efficient volume production process for ultra hard pellet manufacture.

Currently there are 2 main methods described in the literature for forming pellets around a central core of ultra hard material. These methods can generically be called "rotating pan" and "fluidised bed".

The first "rotating pan" method involves introducing the ultra hard core material, e.g. diamond seeds, into either a rotating inclined pan, a drum or any other rotating vessel, where the pellet can be built up by 1) spraying a slurry containing metal powder, binder and solvent (encapsulating or coating material) over the rotating diamond seeds or 2) the binder and solvent is/are sprayed separately and the metal powder then "sprinkled" over the rotating diamond seeds. Rotation of the pan separates the coated diamond seeds (emergent pellets) and allows time for removal of the solvent from the sprayed material to form a concentric jacket of encapsulating material which increases in volume as the process proceeds. This technique is efficient in terms of depositing encapsulating material and thus building up the pellet mass quickly. The difficulty with this method is that it is susceptible to agglomeration of the cores and/or early pellets in the initial stages of the process. Deposition rates must be very slow to avoid agglomeration. This increases the overall processing time and reduces the throughput of the process. Agglomeration reduces in severity after the emergent pellet has attained a critical size.

The consequence of the agglomeration is that the final pellets may have significant size distribution and may contain more than one core per pellet. This contributes to increased process time and cost.

The second method involves using a fluidised bed technique. In this method, the ultra hard cores, e.g. diamond seeds, are suspended in a flow of gas within a chamber, into which a fine suspension of binder, solvent and particulate material (e.g. metal powder) (the encapsulating material) is sprayed. Alternatively, the binder-solvent may be sprayed with separate powder addition. The emergent pellets are built up in volume proportional (non-linearly) to the residence time spent in the chamber. The advantage of this process is that the fluid bed allows a good separation of the core seeds and thereby ensures that a single core (diamond seed) is contained in each pellet while depositing encapsulating material at a reasonable rate.

The disadvantage of this technique is that the maximum deposition rate is relatively slow and when using a high density particulate encapsulating material e.g. Mo, W and WC, the increasing mass of the pellets presents difficulties in terms of the capabilities of the equipment to maintain the suspension. This can be addressed by increasing the capacity of the equipment but this is costly and impacts on the commercial viability of producing commercial volumes of material.

A need exists for a process for the formation of pellets containing an ultra hard core coated (encapsulated) with an encapsulating material which process allows for increased production rates of the pellets and/or improved quality yield of pellets so produced.

### SUMMARY OF THE INVENTION

According to the first aspect of the present invention there is provided a process for the formation of pellets containing a core coated with an encapsulating material, the process including the steps of:
- suspending core material in a flow of gas;
- contacting the core material with encapsulating material to form pellets,
- introducing the pellets into a rotating vessel,
- contacting the pellets with encapsulating material to form pellets of greater mass than the pellets introduced into the rotating vessel.

The encapsulating material used in the gas flow arrangement may be the same or different to the encapsulating material used in the rotating vessel.

Preferably the rotating vessel is a pan or a drum.

Essentially the solution to the problems described above is to combine the two techniques known in the art into a single process design. As such, the initial stages of the process involve a fluid bed approach to maximise the yield of pellets containing one core particle only e.g. diamond seeds. The pellets may be built up to a critical size volume (Vcrit) whilst remaining in a fluid suspension. When the pellets attain this critical size, the pellets are transferred to a rotating pan where the pellets form the (sub) core of the final pellet process. The pellets so produced have a volume significantly greater than the pellets as introduced and the risk of agglomeration is much reduced as the layer on the surface absorbs the spray more quickly and thus deposition rates may be increased. In addition, the weightier particles are less likely to be held together by surface tension of the spray.

Also described is a pellet containing a core coated with an encapsulating material whenever produced by a process as hereinbefore described.

### DESCRIPTION OF THE EMBODIMENTS

The process for the formation of pellets containing an ultra hard core coated with an encapsulating material includes the steps of:
- suspending ultra hard core material in a flow of gas;
- contacting the ultra hard core material with encapsulating material to form pellets,
- introducing the pellets into a rotating vessel,
- contacting the pellets with encapsulating material to form pellets of greater mass than the pellets introduced into the rotating vessel.

The core is preferably comprised of hard core material, most preferably ultra hard core material. The ultra hard core material may be selected from material comprising cubic boron nitride and diamond including natural and synthetic diamond, synthetic diamond including both High Pressure High Temperature (HPHT) and Chemical Vapour Deposition (CVD) synthetic diamond, coated or cladded diamond, boron carbide, boron suboxide or combinations thereof.

The ultra hard core material is preferably suspended in a chamber or work vessel which is preferably a fluidised bed granulating/encapsulating apparatus. The work vessel may be a fluidised bed granulating/encapsulating apparatus of the type having a material work area, a rotatable plate disposed immediately beneath the work area and means for conveying a gaseous fluid through the work area for fluidised circulation of charge material therewithin, the granulating apparatus being operated to generally individually fluidise the ultra hard core material within the work area. It will be appreciated, however, that such a particular arrangement does not lie central to the present invention.

The encapsulating material may be comprised of metal and/or ceramic powder, binder and/or solvent. The metal powder may be cobalt, copper, iron, bronze, tungsten carbide, nickel, tungsten metal, molybdenum, zinc, brass, silver, or a mixture of two or more thereof. The particle size is preferably greater than approximately 0.01 micrometers, preferably greater than 0.1 micrometer, more preferably greater than 0.2 micrometers, more preferably greater than 0.5 micrometers, more preferably greater than 1 micrometers, more preferably greater than 2 micrometers, more preferably greater than 4 micrometers and most preferably greater than 8 micrometers. The particle size of the metal and/or ceramic powder is less than approximately 500 micrometers, more preferably less than 450 micrometers, more preferably less than 350 micrometers, more preferably less than 300 micrometers and most preferably less than 250 micrometers.

The core material is preferably greater than 10 micrometers, more preferably greater than 20 micrometers, more preferably greater than 50 micrometers, more preferably greater than 100 micrometers, more preferably greater than 200 micrometers, more preferably greater than 400 micrometers and most preferably greater than 800 micrometers. The particle size of the ultra hard core material is less than approximately 5000 micrometers, more preferably less than 4500 micrometers, more preferably less than 3500 micrometers, more preferably less than 3000 micrometers and most preferably less than 2500 micrometers

Polyethylene glycol, liquid paraffin, glycerol, shelac, polyvinyl alcohol (PVA), polyvinyl butyral(PVB), cellulose or stearic acid are preferred as the binding agent and the solvent may be water and/or an organic solvent, preferably ethyl alcohol or trichloro-ethylene or isopropyl alcohol (IPA). The metal powder should comprise no greater than approximately 80%, preferably no greater than approximately 70%, preferably no greater than approximately 60%, preferably no greater than approximately 50%, by weight of a slurry and the binder should comprise no greater than approximately 30%, preferably no greater than approximately 25%, preferably no greater than approximately 20%, preferably no greater than approximately 15%, preferably no greater than approximately 10%, preferably no greater than approximately 5% of the weight of the metal powder in the slurry.

In addition, a hard phase may be added to the metal and/or ceramic powder to improve the wear resistance of the encapsulating material itself. This hard phase could be tungsten carbide (WC), particles of WC-cobalt cermet or any conventional ceramic hard phase such as silicon carbide (SiC), silicon nitride (SiN), alumina (Al₂O₃) etc. or mixture of any of these. As above, the size of these hard phases could range from 0.01 microns to 500 microns (micrometers).

In the preferred embodiment of the present method, the spraying of the encapsulating material is continued for a sufficient time to build the coating on each core to achieve a predetermined critical size (Vcrit). The average diametric dimension of each pellet may range up to, but no greater than, approximately 5, preferably no greater than 4, more preferably no greater than 2 times the average diametric dimension of the ultra hard cores. The plate of the fluidised bed granulating apparatus is preferably rotated throughout the course of the granulating operation to circulate the ultra hard cores within the material work area during fluidisation of the cores.

The pellets as produced are thereafter introduced into a rotating, preferably inclined pan, where the pellet can be built further up by 1) spraying a slurry containing metal and/or ceramic powder, binder and solvent (encapsulating material) over the rotating diamond seeds and/or 2) the binder and solvent is/are sprayed separately and the metal and/or ceramic powder then "sprinkled" over the rotating diamond seeds. Rotation of the pan allows time for reduction and possible removal of the solvent from the sprayed encapsulating material to form a concentric jacket of encapsulating material which increases in volume as the process proceeds. The pellets are preferably always wet to a degree; while additional solvent is removed as it is put on. For the avoidance of doubt, the material from the bed is first allowed to be slightly wet before adding powder, then as more solvent/binder is added there is a constant replenishment - hence removal of solvent.

The process according to the present invention results in significantly increased accretion rate in the pan method over use of the pan method alone. According to the teaching of the present invention, the diameter of the pellets can increase by 10 microns per hour, preferably 20 microns per hour, more preferably 50 microns per hour, more preferably 100 microns per hour, more preferably 150 microns per hour, more preferably 200 microns per hour, more preferably 300 microns per hour, more preferably 400 microns per hour, most preferably 450 microns per hour. This results in a much reduced process time in the pan coater and subsequent reduction in process costs.

This advantage is achieved by ensuring the pellets from the fluidised bed granulator are of sufficient volume (Vcrit) to ensure minimal agglomeration in the rotating pan coater in the initial stages, thereby allowing a faster build up rate.

The pelletised material has a broad range of applications including the pelletising of diamond seeds, preferably in the range 200 -1500 microns, with particulate metal including but not limited to Co, Fe, Ni, W, Mn, Cu and Sn, ceramic, tungsten carbide powders and/or aggregates thereof.

The process according to the present invention provides a significant advantage in terms of cost of production of pellets and enables dense metal powders to be used in a commercially viable production process.

The invention will now be described with reference to the following non-limiting examples and figures in which:
Figure 2 illustrates the deposition rates for the 45/50# fraction,
Figure 3 illustrates the deposition rates for the 40/45# fraction,
Figure 4 illustrates the size distribution of the charge of W/Mo encapsulated diamond and the result which was further encapsulated with Fe, and

### Example 1

Diamond was encapsulated with a metal bond on a Dim-Net CT-3000D fluidised bed type diamond coating machine. A slurry was prepared by mixing equal weights (400g) of bond powder (Umicore Cobalite-CNF) and water With 4 weight% (wt%) of the bond powder in PVA. 2,000cts (400g) of SDA100+TC 40/50# diamond was loaded in the coating machine.

The following settings were used:

| | Temp (°C) | Fan |
|---|---|---|
| Inlet | 47 | 90/115 |
| Outlet | 28 | 65/115 |
| Pump | 3/10 | 1mmØ tube |
| Spray | 1.75 | kgf/cm² |

This is the lowest spray rate of the pump, Eyla type MP-1000.

At these settings, the weight of the diamond was increased by 12g in 120 minutes, this is a rate of 6g/hr. There was no agglomeration obviously visible in the charge. The material was returned to the machine and encapsulation was continued at the following settings.

| | Temp (°C) | Fan |
|---|---|---|
| Inlet | 53 | 100/115 |
| Outlet | 28 | 45/115 |
| Pump | 5/10 | 1mmØ tube |
| Spray | 1.6 | kgf/cm² |

As can be seen from the table, the pumping rate was increased by 67%. At these settings, the weight of the diamond was increased by 30g in 120 minutes, this is a rate of 15g/hr. Some agglomeration was seen, this was separated and by weight was 7.25% of the total weight of the charge. This fraction was removed and the rest of the charge returned to the machine where encapsulation was continued at the following settings.

| | Temp (°C) | Fan |
|---|---|---|
| Inlet | 53 | 100/115 |
| Outlet | 28 | 45/115 |
| Pump | 7/10 | 1mmØ tube |
| Spray | 1.5 | kgf/cm² |

Spray rate for this test was further increased by 40% (that is 130% above the first test). At these settings, the weight of the diamond was increased by 40g in 90 minutes, this is a rate of 26.7g/hr. More agglomeration was seen than before, this was separated and by weight was almost 30% of the total weight of the charge.

This example goes to show that using the fluidised bed system at a low rate can result in practically no agglomeration occurring, but, if the rate of deposition is increased too much in the initial stages then agglomeration can occur.

At the start, 600g of the material was charged on the machine but this was soon split into two batches as the machine did not have the airflow capacity to keep this weight fluidised. The details of the runs are shown in Table 1 below. Every two runs, the batches were mixed and then split again to make sure that no single batch was coated more than the other.

**Table 1: Details of runs for Example 2 on the fluidized bed machine.**

| | **Batch** | **Starting weight (g)** | **Finish weight (g)** | **Weight increase (g)** | **Time (hr)** | **Encap rate (g/hr)** | **Pump No.** |
|---|---|---|---|---|---|---|---|
| Run 1 | | 600 | 604 | 4 | 0.75 | 5.3 | 3 |
| Run 2 | | 604 | 612 | 8 | 0.75 | 10.7 | 4 |
| Run 3 | | 610 | 618 | 8 | 1 | 8.0 | 4 |
| Run 4 | A | 300 | 310 | 10 | 1 | 10.0 | 5 |
| Run 5 | B | 312 | 332 | 20 | 2 | 10.0 | 5 |
| Run 6 | A | 318 | 322 | 4 | 0.5 | 8.0 | 5 |
| Run 7 | A | 322 | 342 | 20 | 1.75 | 11.4 | 5 |
| Run 8 | B | 314 | 344 | 30 | 3 | 10.0 | 7 |
| Run 9 | A | 316 | 346 | 30 | 2.25 | 13.3 | 10 |
| Run 10 | B | 344 | 358 | 14 | 1 | 14.0 | 10 |
| Run 11 | A | 344 | 368 | 24 | 2 | 12.0 | 10 |
| Run 12 | B | 358 | 384 | 26 | 1 | 26.0 | 10 |
| Run 13 | A | 368 | 388 | 20 | 1 | 20.0 | 10 |
| Run 14 | B | 384 | 408 | 24 | 1.5 | 16.0 | 10 |
| Run 15 | A | 388 | 408 | 20 | 1 | 20.0 | 10 |
| Run 16 | B | 408 | 422 | 14 | 1.5 | 9.3 | 10 |
| Run 17 | A | 408 | 418 | 10 | 1 | 10.0 | 10 |
| Run 18 | B | 422 | 430 | 8 | 1 | 8.0 | 10 |

### Example 3

For this example, a Kalweka Pelletizer (Type-PLZ by Karnavati Engineering) rotating pan was used to build up more metal powder on partially encapsulated diamond. For this example, 873g of partially encapsulated diamond was placed on the rotating pan. The pan was angled at 45° ±3° and rotated at 30 rpm which brought the partially encapsulated diamond up the pan, allowing it to fall back down again without it being held to the wall by centrifugal forces.

While the pan was rotating, metal powder was added to the charge by using a vibrating dispenser and at the same time spraying a binder solution onto the moving charge.

The metal powder added is the same as already on the charge, i.e 60wt% w/, 40wt% Mo mixture. The binder which was sprayed was a 10 wt% PVA in water. A 5wt% PVA solution, was tried previously but this was not sufficient to allow continuous build-up. The rates at which the powder and binder are added will determine the overall build-up rate. If excess binder solution is sprayed, then the system will appear wet. Oppositely, if less binder is sprayed then it will appear dry. For this example, the system was purposely allowed to appear wet which reduced dust creation.

Encapsulation was continued for 165 minutes. In this time the weight of the charge was increased to 1432g, that is a rate of 203.3g per hour. In addition, this weight of charge could not be fluidised by the fluid bed machine. In the final product, very little in agglomeration could be seen.

### Example 4

For this example, the rotating pan which was used in the Example 3 was again utilised: 874g of partially encapsulated diamond was placed on the rotating pan. The pan was angled at 45° ±3° and rotated at 30 rpm. While the pan was rotating, metal powder (as Example 3) was added to the charge by using a vibrating dispenser and at the same time spraying a binder solution (as Example 3) onto the moving charge. For this example, the system was purposely allowed to appear dry, which did create dust. Encapsulation was continued for 205 minutes. In this time the weight of the charge was increased to 1450g, that is a rate of 168.6g per hour. In addition, this weight of charge could not be fluidised by the fluid bed machine.

### Example 5

504g (2520cts) of SDA100+ 40/50 with a TiC coating was loaded in the rotating pan as described in Example 3. The pan was angled at 45° and rotated at 40rpm. Binder solution was sprayed slowly while adding Umicore Cobalite-CNF slowly. The powder addition was measured at between 0.25g and 0.5g per minute. After an hour of encapsulating, the charge was removed and any agglomerates separated on a vibrating table. Almost 50% of the charge was not single particles. The actual weight increase was 28g, corresponding to 28g/hr. The work was halted at this stage, but it does show how difficult it is to prevent agglomeration on the rotating pan when starting with diamond without an initial encapsulated layer.

### Example 6

This example was to increase 1200cts (240g) of 40/45# and 800cts (160g) 45/50# TiC coated E6 SDB diamond in weight by 10.9 times with an iron powder. The individual half sizes were encapsulated separately. Firstly, the iron was built-up in the fluid bed machine as described in Example 1. This was subsequently transferred to the rotating pan (as described in Example 3) to continue encapsulation. The following settings were used for this test.

| | Temp (°C) | Fan |
|---|---|---|
| Inlet | 45 to 55 | 85 to Max |
| Outlet | 29 to 32 | 20 to 60 |
| Pump | 3 to 5 | 0.8mmØ tube |
| Spray | 2.0 to 4.5 | kgf/cm² |

For the 800cts (160g) 45/50#fraction, the deposition rates are shown in the Figure 2. As can be seen from this figure, there is again about a 10 fold increase in deposition rate on the pan when compared to the fluid bed. The drop in rate was because the powder preferentially granulated in the pan instead of encapsulating on the diamond. This was solved by using a more "sticky" binder solution of 15wt% PVA. At each stage, agglomerates were separated by sieving, at no time was there more than an estimated 5% particles which were not singular.

For the 1200cts (240g) 40/45#fraction, the deposition rates are shown in Figure 3. As can be seen from this figure, there is again about a 10 fold increase in deposition rate on the pan when compared to the fluid bed. At each stage, agglomerates were separated by sieving, at no time was there more than an estimated 5% particles which were not singular.

Not only is the deposition rate faster on the rotating pan, but no slurry needs to be produced and using the machine is much simpler, i.e. there is no air heating, blocking of tubes etc. Overall, it took 17 days to build up on average 1.65 times the weight of starting diamond in iron powder on both half sizes. On the rotating pan, it took 11 days to build up the rest of the iron (9.25 times the original starting wt of the full size) .to achieve the required 10.9 times increase. If the rotating pan was not used, conceivably it would have taken about another 100 days to build up the diamond to the required weight with iron if the material could have been fluidised. Certainly, batch splitting would have to be used.

### Example 7

350g of the same W/Mo partially encapsulated diamond was loaded onto the pan coater as described in Example 3. The pan was angled at 45° and rotated at 32rpm. Onto the moving charge, iron powder, the same as used in Example 6 was added in a controlled manner while spraying a 15wt% binder solution at the same time. As this was a test, the rates at which the powder and binder were added were conservative. Encapsulation was continued for about 1 hour which resulted in the weight increasing to 515g. This is a rate of 165g per hour. The median sizing of the initial W/Mo partially encapsulated was 640um, this was increased to a median of 900um. The size distribution of the original charge and the resulting Fe encapsulated material is shown in the graph of Figure 4 below. This example shows that it is possible to encapsulate more than one material on diamond.

## Claims

1. A process for the formation of pellets containing a core coated with an encapsulating material, the process including the steps of:
- suspending core material in a flow of gas;
- contacting the core material with encapsulating material to form pellets,
- introducing the pellets into a rotating vessel,
- contacting the pellets with encapsulating material to form pellets of greater mass than the pellets introduced into the rotating vessel.

2. A process according to claim 1 wherein the rotating vessel is a pan or a drum.

3. A process according to either one of claims 1 and 2 wherein the core material is ultra hard core material, wherein the ultra hard core material is preferably selected from material comprising cubic boron nitride, diamond including natural and synthetic diamond, synthetic diamond including both High Pressure High Temperature (HPHT) and Chemical Vapour Deposition (CVD) synthetic diamond, and coated or cladded diamond, boron carbide, boron suboxide or combinations thereof.

4. A process according to any previous claim wherein the core material is suspended in a chamber or work vessel which is a fluidised bed granulating/encapsulating apparatus.

5. A process according to claim 4 wherein the work vessel is a fluidised bed granulating/encapsulating apparatus of the type having a material work area, a rotatable plate disposed immediately beneath the work area and means for conveying a gaseous fluid through the work area for fluidised circulation of charge material therewithin, the granulating apparatus being operated to generally individually fluidise the core material within the work area.

6. A process according to any previous claim wherein the encapsulating material is comprised of metal and/or ceramic powder, binder and/or solvent.

7. A process according to claim 6 wherein the metal and/or ceramic powder is cobalt, copper, iron, bronze, tungsten carbide, nickel, tungsten metal, molybdenum, zinc, brass, silver, or a mixture of two or more thereof, and/or wherein a particle size of the metal and/or ceramic powder is greater than 0.1 micrometers, and/or wherein a particle size of the metal and/or ceramic powder is less than 300 micrometers, and/or wherein the binder is selected from polyethylene glycol, liquid paraffin, glycerol, shelac, polyvinyl alcohol (PVA), polyvinyl butyral(PVB), cellulose and/or stearic acid, and/or wherein the solvent is water and/or an organic solvent, and/or wherein the metal and/or ceramic powder comprises no greater than 80% by weight of a slurry, and/or wherein a hard phase is added to the metal powder.

8. A process according to claim 7 wherein the solvent is ethyl alcohol and/or trichloro-ethylene or isopropyl alcohol (IPA).

9. A process according to claim 7 wherein the binder comprises no greater than approximately 30% of the weight of the metal and/or ceramic powder in the slurry.

10. A process according to claim 7 wherein the hard phase is selected from tungsten carbide (WC), particles of WC-cobalt cermet or a conventional ceramic hard phase such as silicon carbide (SiC), silicon nitride (SiN), alumina (Al₂O₃) or mixture of any of these.

11. A process according to claim 7 wherein the size of the hard phase ranges from 0.1 microns to 500 microns.

12. A process according to any previous claim wherein spraying of the encapsulating material is continued for a sufficient time to build the coating on each core to achieve a predetermined critical size (Vcrit) wherein an average diametric dimension of each pellet may range up to, but no greater than, 5 times the average diametric dimension of the ultra hard cores.

13. A process according to any previous claim wherein the pellets are introduced into a rotating pan, where the pellet can be built further up by:
- spraying a slurry containing metal and/or ceramic powder, binder and solvent (encapsulating material) over the rotating diamond seeds; and/or
- the binder and solvent is/are sprayed separately and the metal and/or ceramic powder then "sprinkled" over the rotating diamond seeds.

14. A process according to any previous claim wherein the diameter of the pellets increases by at least 10 microns per hour.

## Patentansprüche

1. Verfahren zur Herstellung von Pellets, die einen mit einkapselndem Material beschichteten Kern enthalten, wobei das Verfahren die Schritte umfasst, dass:
- Kemmaterial in einem Gasstrom suspendiert wird;
- das Kemmaterial mit einkapselndem Material in Kontakt gebracht wird, um Pellets herzustellen,
- die Pellets in ein rotierendes Gefäß eingebracht werden,
- die Pellets mit einkapselndem Material in Kontakt gebracht werden, um Pellets größerer Masse als die Pellets, die in das rotierende Gefäß eingebracht wurden, herzustellen.

2. Verfahren nach Anspruch 1, wobei das rotierende Gefäß eine Wanne oder eine Trommel ist.

3. Verfahren nach einem der Ansprüche 1 und 2, wobei das Kernmaterial ein ultrahartes Kemmaterial ist, wobei das ultraharte Kemmaterial vorzugsweise ausgewählt ist aus Material umfassend kubisches Bornitrid, Diamant einschließlich natürlichem und synthetischem Diamant, synthetischer Diamant einschließlich durch Hochdruck-Hochtemperatursynthese (HPHT) und chemische Gasphasenabscheidung (CVD) hergestellten synthetischen Diamant, und beschichteten oder plattierten Diamant, Borkarbid, Borsuboxid oder Kombinationen daraus.

4. Verfahren nach einem der vorhergehenden Ansprüche, wobei das Kemmaterial in einer Kammer oder einem Arbeilsgefäß suspendiert wird, welche/s eine Wirbelschicht-Granulier-/Verkapselvorrichtung ist.

5. Verfahren nach Anspruch 4, wobei das Arbeitsgefäß eine Wirbelschicht-Granulier-/Verkapselvorrichtung von dem Typ mit einem Materialarbeitsbereich, einer unmittelbar unterhalb des Arbeitsbereichs angeordneten drehbaren Platte und Mittel zur Förderung eines gasförmigen Fluids durch den Arbeitsbereich für die fluidisierte Zirkulation von Chargenmaterial innerhalb desselben ist, wobei die Granuliervorrichtung betrieben wird, um das Kemmaterial innerhalb des Arbeitsbereichs im Allgemeinen einzeln zu fluidisieren.

6. Verfahren nach einem der vorhergehenden Ansprüche, wobei das einkapselnde Material aus Metall- und/oder Keramikpulver, Bindemittel und/oder Lösemittel besteht.

7. Verfahren nach Anspruch 6, wobei das Metall- und/oder Keramikpulver Kobalt, Kupfer, Eisen, Bronze, Wolframkarbid, Nickel, Wolframmetall, Molybdän, Zink, Messing, Silber, oder ein Gemisch aus zwei oder mehr derselben ist, und/oder wobei die Partikelgröße des Metall- und/oder Keramikpulvers größer als 0,1 Mikrometer beträgt, und/oder wobei die Partikelgröße des Metall- und/oder Keramikpulvers kleiner als 300 Mikrometer ist, und/oder wobei das Bindemittel ausgewählt ist aus Polyethylenglykol, flüssiges Paraffin, Glycerin, Schellack, Polyvinylalkohol (PVA), Polyvinylbutyral (PVB), Zellulose und/oder Stearinsäure, und/oder wobei das Lösemittel Wasser und/oder ein organisches Lösemittel ist, und/oder wobei das Metall- und/oder Keramikpulver nicht mehr als 80 Gew.% einer Aufschlämmung umfasst, und/oder wobei eine Hartphase zu dem Metallpulver hinzugefügt wird.

8. Verfahren nach Anspruch 7, wobei das Lösemittel Ethylalkohol und/oder Trichlorethylen oder Isopropylalkohol (IPA) ist.

9. Verfahren nach Anspruch 7, wobei das Bindemittel nicht mehr als ungefähr 30 % des Gewichts des Metall- und/oder Keramikpulvers in der Aufschlämmung umfasst.

10. Verfahren nach Anspruch 7, wobei die Hartphase ausgewählt ist aus Wolframkarbid (WC), Partikel aus WC-Kobalt-Cermet oder einer herkömmlichen Keramikhartphase wie Siliziumkarbid (SiC), Siliziumnitrid (SiN), Aluminiumoxid (Al₂O₃) oder einem beliebigen Gemisch aus diesen.

11. Verfahren nach Anspruch 7, wobei die Größe der Hartphase von 0,1 Mikrometer bis 500 Mikrometer reicht.

12. Verfahren nach einem der vorhergehenden Ansprüche, wobei das Versprühen des einkapselnden Materials für eine Zeit fortgesetzt wird, die ausreicht, um die Beschichtung auf jedem Kem so aufzubauen, dass eine zuvor festgelegte kritische Größe (V_{crit}) erreicht wird, wobei eine mittlere Durchmessergröße jedes Pellets bis zum Fünffachen, aber nicht mehr, der mittleren Durchmessergröße der ultraharten Kerne reicht.

13. Verfahren nach einem der vorhergehenden Ansprüche, wobei die Pellets in eine rotierende Wanne eingebracht werden, wo die Pellets weiter aufgebaut werden können durch:
- Versprühen einer Metall- und/oder Keramikpulver, Bindemittel und Lösemittel (einkapselndes Material) enthaltenden Aufschlämmung über die rotierenden Diamantkeime; und/oder
- das Bindemittel und das Lösemittel werden separat versprüht und das Metall- und/oder Keramikpulver wird dann über die rotierenden Diamantkeime "gestreut".

14. Verfahren nach einem der vorhergehenden Ansprüche, wobei der Durchmesser der Pellets um zumindest 10 Mikrometer pro Stunde zunimmt.

## Revendications

1. Procédé pour la formation de granules contenant un coeur enrobé avec un matériau d'encapsulation, le procédé incluant les étapes de :
- suspension du matériau de coeur dans un flux de gaz,
- mise en contact du matériau de coeur avec le matériau d'encapsulation pour former des granules,
- introduction des granules dans une cuve rotative,
- mise en contact des granules avec le matériau d'encapsulation pour former des granules de masse plus grande que les granules introduits dans la cuve rotative.

2. Procédé selon la revendication 1, dans lequel la cuve rotative est une turbine d'enrobage ou un tambour.

3. Procédé selon l'une ou l'autre des revendications 1 et 2, dans lequel le matériau de coeur est un matériau de coeur ultra dur, dans lequel le matériau de coeur ultra dur est préférablement sélectionné parmi les matériaux comprenant le nitrure de bore cubique, le diamant incluant le diamant naturel et synthétique, le diamant synthétique incluant à la fois le diamant synthétique obtenu par Haute Pression Haute Température (HPHT) et le diamant synthétique obtenu par Dépôt Chimique en Phase Vapeur (CVD), et enrobé ou le diamant revêtu de métal, le carbure de bore, le sous-oxyde de bore ou des combinaisons de ceux-ci.

4. Procédé selon l'une des précédentes revendications, dans lequel le matériau de coeur est suspendu dans une chambre ou une cuve de travail qui est un appareil de granulation/encapsulation en lit fluidisé.

5. Procédé selon la revendication 4, dans lequel la cuve de travail est un appareil de granulation/encapsulation en lit fluidisé du type ayant une surface de travail pour matériaux, une plaque tournante disposée immédiatement sous la surface de travail et des moyens pour convoyer un fluide gazeux à travers la surface de travail pour la circulation fluidisée de la charge des matériaux s'y trouvant, l'appareil de granulation étant actionné pour tluidiser généralement individuellement le matériau de coeur à l'intérieur de la surface de travail.

6. Procédé selon l'une quelconque des revendications précédentes, dans lequel le matériau d'encapsulation est composé de poudre de métal et/ou de céramique, de liant et/ou de solvant.

7. Procédé selon la revendication 6, dans lequel la poudre de métal et/ou de céramique est du cobalt, du cuivre, du fer, du bronze, du carbure de tungstène, du nickel, du tungstène métallique, du molybdène, du zinc, du laiton, de l'argent, ou un mélange de deux ou plus de ces derniers, et/ou dans lequel une taille de particule de poudre de métal et/ou de céramique est supérieure à 0,1 micromètre, et/ou dans lequel une taille de particule de poudre de métal et/ou de céramique est inférieure à 300 micromètres, et/ou dans lequel le liant est choisi parmi le polyoxyéthylèneglycol, la paraffine liquide, le glycérol, la gomme laque, l'alcool polyvinylique (PVA), le polyvinyle de butyral (PVB), la cellulose et/ou l'acide stéarique, et/ou dans lequel le solvant est de l'eau et/ou un solvant organique, et/ou dans lequel la poudre de métal et/ou de céramique ne comporte pas plus de 80% en poids d'une suspension, et/ou dans lequel une phase ultra dure est ajoutée à la poudre de métal.

8. Procédé selon la revendication 7, dans lequel le solvant est de l'alcool éthylique et/ou du trichloréthylène ou de l'alcool d'isopropyle (IPA).

9. Procédé selon la revendication 7, dans lequel le liant ne comporte pas plus d'approximativement 30% du poids de la poudre de métal et/ou de céramique dans la suspension.

10. Procédé selon la revendication 7, dans lequel la phase ultra dure est choisie parmi le carbure de tungstène (WC), les particules de cermet de WC-cobalt ou une phase conventionnelle ultra dure de céramique telle que le carbure de silicium (SiC), le nitrure de silicium (SiN), l'alumine (Al₂O₃) ou un mélange de plusieurs de ceux-ci.

11. Procédé selon la revendication 7, dans lequel la taille de la phase dure varie de 0,1 micron à 500 microns.

12. Procédé selon l'une quelconque des revendications précédentes, dans lequel la pulvérisation du matériau d'cncapsulation se poursuit pendant un temps suffisant pour construire l'enrobage sur chaque coeur pour atteindre une taille critique prédéterminée (Vcrit) dans laquelle la dimension du diamètre de chaque granule peut aller jusqu'à, mais pas plus de, 5 fois la dimension du diamètre moyen des coeurs ultra durs.

13. Procédé selon l'une quelconque des revendications précédentes, dans lequel les granules sont introduits dans turbine d'enrobage rotative, où les granules peuvent se développer davantage par :
- pulvérisation d'une suspension contenant la poudre de métal et/ou de céramique, le liant et le solvant (matériau d'encapsulation) sur les grains de diamant tournants et/ou
- le liant et le solvant est/sont pulvérisé(s) séparément et la poudre de métal et/ou de céramique à ce moment-là « saupoudrée(s) » sur les grains de diamant tournants.

14. Procédé selon l'une quelconque des revendications précédentes, dans lequel le diamètre des granules augmente d'au moins 10 microns par heure.
